

# UNITED STATES PATENT OFFICE.

HARRY ST. L. BUCHNER, OF WOLLASTON, MASSACHUSETTS.

## TEXTILE BELTING AND METHOD OF PREPARING THE SAME.

1,249,019.

Specification of Letters Patent.

Patented Dec. 4, 1917.

No Drawing.

Application filed December 18, 1916. Serial No. 137,716.

To all whom it may concern:

Be it known that I, HARRY ST. L. BUCHNER, a citizen of the United States, residing at Wollaston, in the county of Norfolk and 5 State of Massachusetts, have invented a new and useful Textile Belting and Method of Preparing the Same, of which the following is a specification.

This invention relates to a process of 10 treating belting and other similar products, such as spinning frame tapes, spinning frame bands, cotton-stitched belting, cotton-woven belting, and the like for the purpose of rendering them more durable and more 15 flexible; lubricating the fibers to prevent internal wear and access of moisture; preventing the expansion and contraction due to changes in atmospheric conditions, and producing a surface that will have a tendency to prevent slippage and give more uniform transmission of power.

I have discovered that products of the above mentioned kinds are greatly improved in several respects by certain treatment 25 which I will describe, and I have discovered especially that the wear and breaking down of these products is due largely to the fact that as these products turn around pulleys or the like, often first one way and then the other, their interior particles rub against each other and wear each other out, and that by treating them by this process a very 30 large proportion of their wear can be reduced, also the fibers protected from moisture.

These results I secure by treating the belting or the like with a mixture of two petroleum products, viz: a heavy oil asphalt and 40 a lubricating oil from the same base.

I will describe one particular way of carrying out this process which has proved practical and the best way now known to me. The products used for treating fabrics described above are as follows:

a. Refined oil asphalt having the following specifications:

|                                                   |              |
|---------------------------------------------------|--------------|
| Specific gravity at 60°                           | .99-103      |
| Melting point                                     | 115°-130° F. |
| 50 Ductility in centimeters                       | 150          |
| Penetration at 77° F. (in tenths of a millimeter) | 120-140      |
| Penetration at 32° F. (in tenths of a millimeter) | 42           |
| 55 Penetration at 115° F.                         | Too soft     |

|                                |              |
|--------------------------------|--------------|
| Evaporation—7 hours at 325° F. | 1.5%-2.5%    |
| Flash (Cleveland open cup)     | 420°-470° F. |
| Fire test                      | 520°-560° F. |
| Sol. car. bisulfid             | 99%          |
| Sol. car. tetra ben            | 60           |
| Sol. 88 Bé. Penn. naphtha      | 73-79%       |

b. Refined asphaltic base lubricating oil having approximately the following specification:

|                 |         |
|-----------------|---------|
| Gravity         | .19     |
| Flash           | 320° F. |
| Fire test       | 380° F. |
| Vis. at 100° F. | 300' 70 |

A homogeneous mixture of substantially equal quantities by weight of the above mentioned products is made by heating the mixture to a temperature of approximately 200° F. At the same time the products are agitated so that they will be thoroughly assimilated. This gives a compounded product having a viscosity of approximately 190" to 200' at 210° F.

The belting or tapes or other textile products in a dry state are immersed in a bath containing this mixture thinned, preferably by heating up to the temperature above specified, and after being allowed to remain a sufficient time at that temperature to secure a perfect penetration they are then put through rollers having a sufficient pressure to squeeze out the excess material. The thickness and hardness of the strands of the 90 textile material determines the length of time necessary to secure complete saturation. For instance, cotton fibers having a very hard twist and closely woven take a longer time than a loosely twisted, loosely 95 woven fabric.

Then the belt or the like is coated with any suitable finishing material, such as ordinary paint. This serves as means for retaining the saturating compound in and on 100 the fabric and eliminates stickiness of surface until the time same is put in service. It also gives it a better appearance. It is to be remembered that the material I use for coating is not capable of penetrating 105 thoroughly into the fabric. It however leaves the surface in condition so that the finished product can be handled without difficulty.

The mixture of two petroleum asphaltic 110

base products one heavy and the other light substantially as specified above is an important feature of this invention, because, although thoroughly mixed, still the light one retains its penetrative powers and carries the heavier and more stable component with it into the most remote interstices of the fabric. The heavier substance also holds some of the other one with it so that no material difference is seen in the composition at the surface and interior thereof. By using two products from the same asphaltic base there is sufficient affinity between them so that no tendency toward separation of the two ingredients is observed. I have found in practice that a belt so treated is more durable as well as flexible, than one treated with tar or linseed oil mixture, or the like in the ordinary way.

20 Although I prefer to use lubricating oil substantially as specified above for the purpose of diluting the base material, it is possible also to use other petroleum distillates. Of course, the particular asphalt mentioned above may be replaced by substantially equivalent asphalt of other densities within the scope of this invention. Therefore I do not wish to be limited to the precise composition as specified, but what

25 I claim is:—

30 1. The method of treating textile belting, driving tapes and bands, and the like, which consists in saturating the same with a mix-

ture of oil asphalt and refined petroleum distillate.

2. The method of treating textile belting, driving tapes and bands, and the like, which consists in saturating the same with a mixture of refined oil asphalt and refined asphaltic base lubricating oil in substantially equal proportions by weight.

3. The method of treating textile belting, driving tapes and bands, and the like, which consists in saturating the same with a mixture of refined oil asphalt and refined petroleum distillate, in substantially equal proportions by weight, removing the excess and painting the surface.

4. The method of treating textile belting, driving tapes and bands, and the like, which consists in saturating the same with a mixture of oil asphalt and asphaltic base lubricating oil by immersing therein while heated to a temperature of about 200° F.

5. As an article of manufacture, a belt of textile material having its fibers saturated with a mixture of refined oil asphalt and refined asphaltic base lubricating oil.

6. As an article of manufacture, a belt of textile material having its fibers impregnated with a mixture of refined oil asphalt and a petroleum distillate.

In testimony whereof I have hereunto affixed my signature.

HARRY ST. L. BUCHNER